

E. D. LYON, Jr.  
Piles for Railroad-Rails.

No. 150,172.

Patented April 28, 1874.

Fig. 1



Fig. 2.



WITNESSES

*E. T. Bates*  
*Wm. G. Chaffee*

INVENTOR

*E. D. Lyon Jr.*  
per  
*J. C. Lathrop*

ATTORNEY

# UNITED STATES PATENT OFFICE.

EDWIN D. LYON, JR., OF SANDUSKY, OHIO, ASSIGNOR OF TWO-THIRDS HIS  
RIGHT TO F. W. ALVORD AND VOLTARE SCOTT, OF SAME PLACE.

## IMPROVEMENT IN PILES FOR RAILROAD-RAILS.

Specification forming part of Letters Patent No. 150,172, dated April 28, 1874; application filed  
March 24, 1874.

*To all whom it may concern:*

Be it known that I, EDWIN D. LYON, Jr., of Sandusky, in the county of Erie and State of Ohio, have invented certain new and useful Improvements in the Manufacture of Railroad-Rails; and I do hereby declare that the following is a full, clear, and exact description thereof, which will enable others skilled in the art to which it pertains to make and use the same, reference being had to the accompanying drawings, and to the letters of reference marked thereon, which form a part of this specification.

My invention relates to the manufacture of steel-capped rails; and it consists in a peculiarly constructed pile or fagot, from which is obtained, by rolling, an iron rail with a steel-cap covering the top and sides of the head of the rail, and united thereto by a longitudinal dovetail.

In the accompanying drawing, Figure 1 is a transverse vertical section of the fagot, and Fig. 2 is a transverse vertical section of the completed rail.

I build my pile as follows: B B are two old rails cut the required length of the pile, and placed side by side. A is a rolled piece of damper or puddler steel, rolled in the shape shown, so as to fit between the heads of the rails B B, and also on top of the same. Below the steel piece A, and extending down to the base of the rails B B, is a solid piece of iron, C, obtained from the crop end of the rail at the saws; or, in other words, as soon as a rail is made and sawed the required length, I take the crop ends, which generally run over three feet, pass through a small pair of butt-rolls twice, and the piece C is made, thus saving reheating to do this. The rails B B rest upon flat pieces D D and E E, which are made from old rails cut the required length, placed in a furnace as many as five tons at once, heated to a cherry color, and by the aid of a small

break-down roll the pieces required are produced quickly and at slight cost. The whole rests upon a flange-piece, F, rolled from common iron. This pile being carried through the ordinary process, produces a steel-capped rail of the form shown in Fig. 2, G being the rail proper, and H the steel cap covering the top and sides of the head of the rail, and united thereto by a dovetail, a, so that the iron firmly clinches the steel, and will hold it secure in spite of expansion and contraction. This rail also forms a reversible rail, which, when placed on a curve, and the steel worn on one side, can be turned around and thus perform double service. In the construction of the pile, there is an opening, x, in the middle, which enables the heat to penetrate the pile, and the middle thereby gets hot as quick as the outside of the pile, whereby a great saving in coal is effected.

As I do not use "tops and bottoms," or reheated flats, a very large saving in labor and material is effected.

The damper-steel A may be made in any rolling-mill without any change being made in the puddling-furnace, and at the same price as common puddled iron.

Having thus fully described my invention, what I claim as new, and desire to secure by Letters Patent, is—

In the manufacture of steel-capped rails, the construction of the pile or fagot of cap-piece A of steel or puddled iron rails B B, crop ends C, flat pieces D D and E E, and flange-piece F, arranged substantially as herein shown and described, and for the purposes set forth.

In testimony that I claim the foregoing as my own I affix my signature in presence of two witnesses.

EDWIN D. LYON, JR.

Witnesses:

J. TYLER POWELL,  
J. C. LATHROP.